

[54] DIRECT POSITIVE SILVER HALIDE  
PHOTOGRAPHIC EMULSION

[75] Inventors: **Keisuke Shiba; Masanao Hinata; Reiichi Ohi; Arkira Sato; Koutarou Yamasue**, all of Minami-Ashigara, Japan; **Tokiharu Kondo**, deceased, late of Minami-Ashigara, Japan, by Yoshiharu Kondo, legal representative

[73] Assignee: **Fuji Photo Film Co., Ltd.**, Minami-Ashigara, Japan

[22] Filed: **Aug. 21, 1973**

[21] Appl. No.: **390,264**

## Related U.S. Application Data

[63] Continuation-in-part of Ser. No. 149,272, June 2, 1971, abandoned.

## [30] Foreign Application Priority Data

|              |               |          |
|--------------|---------------|----------|
| June 2, 1970 | Japan .....   | 45-47380 |
| June 2, 1971 | Japan .....   | 46-18670 |
| June 2, 1971 | Germany ..... | 2127346  |
| June 2, 1971 | France .....  | 71.19938 |
| June 2, 1971 | Canada .....  | 114642   |
| June 2, 1971 | Belgium ..... | 104148   |

[52] U.S. Cl. .... **96/126; 96/101; 96/131; 96/133; 96/142**

[51] Int. Cl. .... **G03c 1/14**

[58] Field of Search .... **96/126, 101**

## [56] References Cited

## UNITED STATES PATENTS

|           |         |                   |        |
|-----------|---------|-------------------|--------|
| 3,537,858 | 11/1970 | Wise .....        | 96/126 |
| 3,615,613 | 10/1971 | Shiba et al. .... | 96/126 |
| 3,617,295 | 11/1971 | Shiba et al. .... | 96/126 |
| 3,635,721 | 1/1972  | Sato et al. ....  | 96/126 |

Primary Examiner—J. Travis Brown

Attorney, Agent, or Firm—Sughrue, Rothwell, Mion, Zinn and Macpeak

## [57] ABSTRACT

A direct positive silver halide photographic emulsion containing a combination of at least one halogen accepting cyanine sensitizing dye and at least one compound represented by the formula:



The moieties set out above are specifically defined in the specification.

15 Claims, 2 Drawing Figures

PATENTED JUN 3 1975

3,887,380

FIG. 1



FIG. 2

INVENTORS

KEISUKE SHIBA  
MASANAO HINATA  
REIICHI OHI  
TOKIHARU KONDO  
AKIRA SATO  
KOUTAROU YAMASUE

BY *Sughrue, Rothwell, Mion,  
Zinn & Macpeak*

ATTORNEYS

**DIRECT POSITIVE SILVER HALIDE  
PHOTOGRAPHIC EMULSION**  
**CROSS-REFERENCE TO RELATED  
APPLICATIONS**

This application is a continuation-in-part application of copending application, Ser. No. 149,272, filed June 2, 1971, now abandoned.

**BACKGROUND OF THE INVENTION**

**1. Field of the Invention**

The present invention relates to a silver halide photographic emulsion and especially to a direct positive silver halide photographic emulsion which is fogged previously.

**2. Description of the Prior Art**

When silver halide photographic materials are exposed to light which includes rays in a range of a sensitizing wave length and developed, the silver density increases as the exposure amount increases and reaches to the maximum value. But when the exposure amount further increases, the silver density decreases again to form finally a positive image. Such phenomenon is called generally "Solarization." The same inversion phenomenon as that caused by light is observed in a silver halide which is fogged optically or chemically at preparation thereof.

It is known from U.S. Pat. No. 2,323,187 and Japanese Patent Publication No. 4125/68 that some increase of reversal sensitivity and expansion of a reversal sensitizing wave length range are observed when sensitizing dyes which show a sensitizing function to the common negative-positive type emulsion such as cyanine dyes are added.

It is an important technique in preparation of a direct positive photosensitive material having high sensitivity or a direct positive photosensitive material for color photography to increase further the spectral sensitivity of the direct positive emulsion which is spectrally sensitized by the cyanine dyes.

An object of the present invention is to provide a di-

increases by adding a compound represented by the following formula to the direct positive silver halide emulsion spectrally sensitized by a cyanine dye Formula (II)



wherein Y represents =CH— or =N—, R<sub>2</sub>, R<sub>3</sub>, R<sub>4</sub> and R<sub>5</sub> each represents a hydrogen atom, hydroxyl group,

15 alkoxy group, aryloxy group (e.g. phenoxy group, o-tolyloxy group, p-sulfophenoxy group and  $\beta$ -naphthoxy group), halogen atom (e.g. chlorine atom and bromine atom), heterocyclic nucleus (e.g. morpholinyl group and pyperidyl group), alkylthio group (e.g. methylthio group and ethylthio group), heterocyclithio group (e.g. benzothiazylthio group), arylthio group (e.g. phenylthio group and tolylthio group), amino group, alkylamino group (e.g. methylamino group, ethylamino group, propylamino group, dimethylamino group, diethylamino group, dodecylamino group, cyclohexylamino group,  $\beta$ -hydroxyethylamino group, di- $\beta$ -hydroxyethylamino group and  $\beta$ -sulfoethylamino group), arylamino group or substituted arylamino group (e.g. anilino group, o-sulfoanilino group, m-sulfoanilino group, p-sulfoanilino group, o-anisylamino group, m-anisylamino group, p-anisylamino group, o-toluidino group, m-toluidino group, p-toluidino group, o-carboxyanilino group, m-carboxyanilino group, p-carboxyanilino group, hydroxyanilino group, naphthylamino group and sulfonaphthylamino group), heterocycllamino group (e.g. 2-benzothiazoleamino group and 2-pyridylamino group), aryl group (e.g. phenyl group) and mercapto group, and —A— represents a group selected from the following —A<sub>1</sub>— and

20 —A<sub>2</sub>—.

—A<sub>1</sub>—:



wherein M represents a hydrogen atom or cation which affords water solubility.

—A<sub>2</sub>—:



rect positive silver halide emulsion containing cyanine dyes, the spectral sensitivity of which is markedly increased.

**SUMMARY OF THE INVENTION**

We have found the spectral sensitivity remarkably

But when —A— represents —A<sub>2</sub>—, at least one of R<sub>2</sub>, R<sub>3</sub>, R<sub>4</sub> or R<sub>5</sub> is a substituent having an —SO<sub>3</sub>M group (M has the same meaning as described above).

## BRIEF DESCRIPTION OF THE DRAWINGS

FIG. 1 and FIG. 2 show characteristic curves.

## DETAILED DESCRIPTION OF THE INVENTION

As the cyanine dyes, any dye may be used if it is effective to the common negative-positive type silver halide emulsion, i.e., halogen accepting sensitizing cyanine dyes. But halogen accepting sensitizing cyanine dyes represented by the following formula (I) are particularly preferable.



wherein  $Z$  and  $Z_1$  each represents non-metal atom groups necessary to complete a 5- or 6-member heterocyclic nucleus (which may be substituted in other positions excepting the N-position),  $L_1$ ,  $L_2$  and  $L_3$  each represents a substituted methine group or methine group,  $R$  and  $R_1$  each represents an alkyl group, a substituted alkyl group, an aryl group and a substituted aryl group,  $p$  and  $q$  represent each 1 or 2,  $n$  represents 1, 2 or 3, and  $m$  represents 1 or 2. When  $m=1$ , the formula (I) forms betainecyanine dyes.  $X^-$  represents an anion.

The heterocyclic nuclei formed by  $Z$  and  $Z_1$  include for example, thiazole nuclei such as thiazole, 4-methylthiazole, 4-phenylthiazole, 5-methylthiazole, 5-phenylthiazole, 4,5-dimethylthiazole, 4,5-

diphenylthiazole, 4-(2-thienyl)-thiazole, benzothiazole, 4-chlorobenzothiazole, 5-chlorobenzothiazole, 6-chlorobenzothiazole, 7-chlorobenzothiazole, 5-methylbenzothiazole, 6-methylbenzothiazole, 5-bromobenzothiazole, 5-phenylbenzothiazole, 5-methoxybenzothiazole, 6-methoxybenzothiazole, 5-ethoxybenzothiazole, 5,6-dimethoxybenzothiazole, 5-

hydroxybenzothiazole, 6-hydroxybenzothiazole, naphtho(1,2)-thiazole, naphtho(2,3)-thiazole and naphtho(2,1)-thiazole; oxazole nuclei such as 4-methyloxazole, 5-methyloxazole, 4-phenyloxazole, 4,5-diphenyloxazole, 4-ethyloxazole, 4,5-dimethyloxazole, 5-phenyloxazole, benzoxazole, 5-chlorobenzoxazole, 5-methylbenzoxazole, 5-phenylbenzoxazole, 6-methylbenzoxazole, 5,6-dimethylbenzoxazole, 5-methoxybenzoxazole, 5-ethoxybenzoxazole, 5-hydroxybenzoxazole, 6-hydroxybenzoxazole, naphtho(1,2)-oxazole, naphtho(2,3)-oxazole and naphtho(2,1)-oxazole; selenazole nuclei such as 4-methylselenazole, 4-phenylselenazole, benzoselenazole, 5-chlorobenzoselenazole, 5-

methylbenzoselenazole, 5-methoxybenzoselenazole, 5-hydroxybenzoselenazole, 5-phenylbenzoselenazole, naphtho(1,2)-selenazole and naphtho(2,1)-selenazole; thiazoline nuclei such as thiazoline and 4-methylthiazoline; oxazoline nuclei such as oxazoline; quinoline nuclei such as 2-quinoline nuclei, e.g. quinoline, 3-methylquinoline, 5-methylquinoline, 8-methylquinoline, 6-chloroquinoline, 8-chloroquinoline, 6-methoxyquinoline, 6-ethoxyquinoline, 6-hydroxyquinoline and 8-hydroxyquinoline, 4-quinoline nuclei, e.g. quinoline, 6-methoxyquinoline, 8-methylquinoline, 6-chloroquinoline, 8-chloroquinoline, 6-fluoroquinoline, 8-fluoroquinoline, 6-hydroxyquinoline, 8-hydroxyquinoline and 6-methylquinoline, 1-isoquinoline nuclei, e.g. isoquinoline and 3,4-

dihydroquinoline, and 3-isoquinoline nuclei e.g. isoquinoline; benzimidazole nuclei such as 1,3-diethylbenzimidazole, 1,3-diethyl-5-chlorobenzimidazole, 1,3-diethyl-5,6-dichlorobenzimidazole and 1-ethyl-3-phenylbenzimidazole; and 3,3'-dialkylindolenine nuclei such as 3,3'-dimethylindolenine, 3,3'-5-trimethylindolenine and 3,3'-7-trimethylindolenine.

Examples of substituted methine for  $L_1$ ,  $L_2$  and  $L_3$  are represented by the following groups and formulae:



$=C(-CH_2C_6H_5)-, =C(-C_6H_5)-, =C(-alkoxy)-, =C(aryloxy)-, =C(-S-alkyl)-, =C(-O-acyl)-, =C(-amido)-, =C(-Cl)-$  and  $=C(-Br)-$ , and substituents in either two methine groups among  $L_1$ ,  $L_2$  and  $L_3$  may bind each other to form a ring represented by the following formula



wherein  $R_6$  represents a hydrogen atom or methyl group, and  $R_7$  represents a hydrogen atom, an alkyl, substituted alkyl, aralkyl, phenyl, substituted alkyl or furyl group.

Alkyl groups in  $R$  and  $R_1$  include, for example, methyl, ethyl, propyl, isopropyl, butyl, hexyl, cyclohexyl, decyl and dodecyl groups.

Substituted alkyl groups in  $R$  and  $R_1$  include, for example, hydroxy alkyl (e.g. 2-hydroxyethyl, 3-hydroxypropyl), alkoxy alkyl (e.g. 2-methoxyethyl), acetoxy alkyl (e.g. 62-acetoxyethyl,  $\gamma$ -acetoxypropyl), carboxy radical-containing alkyl (e.g. carboxymethyl, 2-carboxyethyl, 3-carboxypropyl, 2-(2-carboxyethoxy)ethyl, p-carboxy benzyl), sulfo radical-containing alkyl (e.g. 2-sulfoethyl, 3-sulfopropyl, 4-sulfobutyl, 2-hydroxy-1-sulfopropyl, 2-(3-sulfopropoxy)ethyl, 2-acetoxy-1-sulfopropyl, 3-methoxy-2-(3-sulfopropoxy)propyl, 2-(2-(3-sulfopropoxy)ethoxy)ethyl, 2-hydroxy-3-(3'-sulfopropoxy)-propyl, p-sulfobenzyl, p-sulfophenethyl) aralkyl (e.g. benzyl, phenylethyl) and allyl group.

Aryl groups for  $R$  and  $R_1$  include, for example, phenyl, tolyl, naphthyl, methoxyphenyl and chlorophenyl groups.

Anions of  $X$  include, for example, a chlorine ion, bromine ion, iodine ion, thiocyanic ion, sulfonic ion, perchloric ion, p-toluenesulfonic ion, methylsulfuric ion and ethylsulfuric ion.

Though emulsifying and physical ripening of the silver halide emulsion used in the present invention can be practiced by the same method as in the common emulsions, it is more effective to add salts of a metal of Group VIII of the Periodic Table, such as an iridium salt and a rhodium salt at precipitation or during physical ripening.

In case of sensitizing an emulsion containing a rhodium salt by cyanine dyes, more advantageous reversal

spectral sensitization is performed as compared with the case that an emulsion which does not contain a rhodium salt is sensitized by a combination of cyanine dyes and desensitizing compounds such as Pinakryptol yellow.

The technique of increasing the spectral sensitivity by using compounds represented by the formula (II) together with cyanine dyes can be applied to an emulsion in which rhodium salts are not used, by which further high sensitivity can be obtained as compared with the case of spectral sensitization by using only cyanine dyes.

On the other hand, there is a disadvantage that addition of the cyanine dyes at sensitization of the direct positive silver halide emulsion causes increase of "re-inversion" and enhances the minimum density (D<sub>min</sub>), and consequently, satisfactory whiteness is not obtained sometimes. This phenomenon has a tendency to increase as the amount of the cyanine dyes increases. Herein, re-inversion means the fact that the density increases again after the decrease thereof on the characteristic curve as shown by a dotted line in FIG. 1, although re-inversion depends upon a process for preparing the silver halide photographic emulsion, desensitizing compounds such as Pinacryptol yellow are effective for lowering re-inversion and the minimum density (D<sub>min</sub>). However, when Pinacryptol yellow coexists with a cyanine dye in the direct positive silver halide emulsion sensitized by the cyanine dye, there is a disadvantage that the reversal spectral sensitivity also decreases though the re-inversion and the minimum density (D<sub>min</sub>) is lowered. However, if the compounds represented by the formula (II) used in the present invention coexist with cyanine dyes, not only is the reversal sensitivity increased but the re-inversion and the minimum density is lowered.

It is preferable usually that the cyanine dyes and the compounds represented by the formula (II) are added to an emulsion as a solution respectively. As the solvent

for the cyanine dyes, methanol, ethanol and water are used. As the solvent for the compounds represented by the formula (II), water, methanol and ethanol are used and, if desired, alkali such as caustic soda is added thereto.

An amount of the cyanine dyes added to the direct positive silver halide photographic emulsion is 1-200 mg and preferably 10-100 mg per 1 kg of the emulsion. An amount of the compounds represented by the formula (II) is 5-2000 mg and preferably 10-1000 mg per 1 kg of the emulsion. A preferable ratio by weight of cyanine dyes to compounds (II) is 1:5-1:50.

As the silver halide emulsion used in the present invention, there are silver chloride, silver bromide, silver chloride bromide, silver chloride iodide, silver bromide iodide and silver chloride bromide iodide. The silver halides used in the present invention are fogged to the maximum density by light or a chemical fogging agent. The chemical fogging agent should fog the silver halides without having an adverse influence upon the emulsion. Such chemical fogging agents used include thiourea dioxide, stannous chloride, formaldehyde and hydrazine etc.

After the fogging operation, the pH and pAg are, if desired, adjusted, and a solution of the cyanine dyes is added to the emulsion. Then a solution of the compounds represented by the formula (II) is added. After stirring well the solution is applied to a support. Any of the cyanine dyes and the compounds represented by the formula (II) may precede at addition to the emulsion. A mixture of both of them may be added to the emulsion or may be added during ageing after rinsing. Additives usually used, such as a coating assistant and a hardener, may be added to the emulsion. Further, the direct positive emulsion of the present invention is effectively used together with color couplers. For example, couplers represented by the following structural formulae are used. All of these compounds are well known.

Examples of yellow couplers:

(1)



(2)



(3)



Examples of magenta couplers:

(4)



(5)



(6)



(7)



(8)



(9)



(10)



Examples of cyan couplers:

20 (11)



30 (12)



40 (13)



50 (14)



60

(15)



(16)



As the support, glass, films of cellulose derivatives, films of synthetic resins, baryta paper, water-resistant paper and laminated paper can be preferably used.

In the following, compounds represented by the formula (I) are exemplified.

I - 1



I - 2



I - 3



I - 4



I - 5



I - 6



20 I - 7



25



30



35



40



45



I - 13



I - 14



I - 15



I - 16



I - 17



I - 18



I - 19



I - 20



I - 21



I - 22



I - 23



I - 24



I - 25



I - 26



In the following, compounds represented by the formula (II) are exemplified.

25

Compound II - 1



Compound II - 2



Compound II - 3



Compound II - 4



Compound II - 5



Compound II - 6



Compound II - 7



Compound II - 8



Compound II - 9



Compound II - 10



Compound II - 11



Compound II - 12



Compound II - 13



Compound II - 14



Compound II - 15



Compound II - 16



Compound II - 17



Compound II - 18



Compound II - 19



Compound II - 20



Compound II - 21



Compound II - 22



Compound II - 23



Compound II - 24



The couplers represented by the formula (II) used in the present invention are described in Jap. Pub. No. 10773/68.

In the following, examples of the present invention

fixed by a fixing solution containing thiosulfate, rinsing and drying. Determination of the optical density was carried out by a densitometer. In the following, the results are shown in Table 1.

Table 1

| Experiment No. | Compound Having Formula (I)<br>Amount (mg/kg Em) | Compound Having Formula (II)<br>Amount (mg/kg Em) |
|----------------|--------------------------------------------------|---------------------------------------------------|
| 1              | I - 2                                            | (19.7)                                            |
| 2              | I - 2                                            | ( " )                                             |
| 3              | I - 2                                            | ( " )                                             |
| 4              | I - 2                                            | ( " )                                             |
| 5              | I - 2                                            | ( " )                                             |
| 6              | I - 2                                            | ( " )                                             |
| 7              | I - 2                                            | ( " )                                             |
| 8              | I - 2                                            | ( " )                                             |
| 9              | I - 2                                            | ( " )                                             |
| 10             | I - 6                                            | (19.4)                                            |
| 11             | I - 6                                            | ( " )                                             |
| 12             | I - 6                                            | ( " )                                             |
| 13             | I - 6                                            | ( " )                                             |
| 14             | I - 6                                            | ( " )                                             |
| 15             | I - 6                                            | ( " )                                             |
| 16             | I - 6                                            | ( " )                                             |
| 17             | I - 6                                            | ( " )                                             |
| 18             | I - 6                                            | ( " )                                             |
| 19             | I - 6                                            | ( " )                                             |
| 20             | I - 11                                           | (19.4)                                            |
| 21             | I - 11                                           | ( " )                                             |
| 22             | I - 11                                           | ( " )                                             |
| 23             | I - 11                                           | ( " )                                             |
| 24             | I - 11                                           | ( " )                                             |

are shown. However, the present invention is not limited in these examples.

#### EXAMPLE 1

A silver chloride iodide bromide emulsion (iodine: 35 1.3 mol %, and bromine: 21.3 mol %) was fogged by formalin. The pH and pAg were adjusted to 5.6 and 6.7 respectively. To this emulsion, dyes represented by the formula (I) shown in the following Table 1 were added and mixed homogeneously. Compounds represented by 40 the formula (II) were then added. After mixing the mixture was applied to a triacetyl cellulose base. In order to compare, dyes represented by the formula (I) were added solely to the above-mentioned fogged emulsion and the resulting mixture was applied to a base. After 45 drying, these films were exposed to light through step-wedges by a sensitometer. Yellow sensitivity was determined using a Fuji Filter No. 12.

After exposing to light the films were developed with a developing solution having the following formulation. 50

| Yellow Sensitivity (relative value) | Maximum Density (D max) | Minimum Density (D min) |
|-------------------------------------|-------------------------|-------------------------|
| 100                                 | 2.1                     | 0.74                    |
| 155                                 | 2.0                     | 0.26                    |
| 170                                 | 2.0                     | 0.26                    |
| 130                                 | 2.0                     | 0.25                    |
| 2400                                | 2.0                     | 0.07                    |
| 1800                                | 2.0                     | 0.09                    |
| 1660                                | 2.0                     | 0.09                    |
| 200                                 | 2.0                     | 0.21                    |
| 3100                                | 2.1                     | 0.06                    |
| 100                                 | 2.2                     | 0.56                    |
| 2890                                | 2.2                     | 0.08                    |
| 1200                                | 2.1                     | 0.12                    |
| 650                                 | 2.2                     | 0.21                    |
| 1600                                | 2.2                     | 0.12                    |
| 205                                 | 2.2                     | 0.35                    |
| 300                                 | 2.2                     | 0.30                    |
| 580                                 | 2.2                     | 0.22                    |
| 660                                 | 2.2                     | 0.21                    |
| 1120                                | 2.1                     | 0.15                    |
| 100                                 | 2.1                     | 0.26                    |
| 195                                 | 2.1                     | 0.15                    |
| 1180                                | 2.1                     | 0.08                    |
| 166                                 | 2.1                     | 0.15                    |
| 250                                 | 2.0                     | 0.15                    |

| Experiment No. | Compound Having Formula (I)<br>Amount (mg/kg Em) | Compound Having Formula (II)<br>Amount (mg/kg Em) |
|----------------|--------------------------------------------------|---------------------------------------------------|
| 25             | I - 11                                           | (19.4)                                            |
| 26             | I - 11                                           | ( " )                                             |
| 27             | I - 11                                           | ( " )                                             |
| 28             | I - 11                                           | ( " )                                             |

#### Formulation of the Developing Solution:

|                                         |     |   |
|-----------------------------------------|-----|---|
| Metol                                   | 4   | g |
| Hydroquinone                            | 10  | g |
| Anhydrous Sodium Sulfite                | 60  | g |
| Anhydrous Sodium Carbonate              | 2.5 | g |
| Water is added so as to become 1 liter. |     |   |

After developing, the direct positive images were

| Yellow Sensitivity (relative value) | Maximum Density (D max) | Minimum Density (D min) |
|-------------------------------------|-------------------------|-------------------------|
| 205                                 | 2.1                     | 0.16                    |
| 135                                 | 2.1                     | 0.16                    |
| 120                                 | 2.1                     | 0.16                    |
| 125                                 | 2.1                     | 0.16                    |

## EXAMPLE 2

An emulsion was prepared from the following formulations.

|    |                |      |   |       |
|----|----------------|------|---|-------|
| I  | Gelatin        | 500  | g | liter |
|    | Water          | 10   |   |       |
| II | Silver Nitrate | 1000 | g | liter |
|    | Water          | 10   | g | liter |

added to the above mentioned emulsion followed by adding a hardener and a coating assistant. The products were applied to baryta paper. After drying, these sensitive layers were exposed through step-wedges by a sensitometer. After exposing the sensitive layers were treated by the same procedure as in Example 1. Results were shown in Table 2.

Table 2

| Experiment No. | Compound Having Formula (I) | Compound Having Formula (II) |
|----------------|-----------------------------|------------------------------|
|                | Amount (mg/kg emulsion)     | Amount (mg/kg emulsion)      |
| 29             | I - 1                       | (17.8)                       |
| 30             | I - 1                       | (17.8)                       |
| 31             | I - 1                       | (17.8)                       |
| 32             | I - 3                       | (20.7)                       |
| 33             | I - 3                       | (20.7)                       |
| 34             | I - 3                       | (20.7)                       |
| 35             | I - 4                       | (17.3)                       |
| 36             | I - 4                       | (17.3)                       |
| 37             | I - 4                       | (17.3)                       |
| 38             | I - 5                       | (18.4)                       |
| 39             | I - 5                       | (18.4)                       |
| 40             | I - 5                       | (18.4)                       |
| 41             | I - 7                       | (22.4)                       |
| 42             | I - 7                       | (22.4)                       |
| 43             | I - 7                       | (22.4)                       |
| 44             | I - 8                       | (23.4)                       |
| 45             | I - 8                       | (23.4)                       |
| 46             | I - 8                       | (23.4)                       |
| 47             | I - 9                       | (24.5)                       |
| 48             | I - 9                       | (24.5)                       |
| 49             | I - 9                       | (24.5)                       |
| 50             | I - 10                      | (18.3)                       |

|     |                                                |      |    |       |
|-----|------------------------------------------------|------|----|-------|
| III | Sodium Chloride                                | 350  | g  | ml    |
|     | 0.1% $(\text{NH}_4)_3(\text{RhCl}_6)$ Solution | 200  | ml |       |
|     | Water                                          | 2    | g  | liter |
| IV  | Gelatin                                        | 1700 | g  |       |
|     | Potassium Iodide                               | 12.7 | g  |       |
|     | Water                                          | 7500 | ml |       |

The Solution III was added to the Solution I at 40°C with stirring and then adding the Solution II thereto. After 20 minutes, the Solution IV was added and the pH was adjusted to 9.0 by adding an alkali. The emulsion was fogged by hydrazine dihydrochloride. In this emulsion, the pH and pAg were adjusted to 5.6 and 6.7, respectively. Dyes represented by the formula (I) shown in the following Table 2 were admixed with the above mentioned emulsion. Compounds represented by the formula (II) were then added thereto, followed by adding a hardener and a coating assistant thereto. The products were applied to a baryta paper. In order to compare, dyes represented by the formula (I) were

| Experiment No. | Yellow Sensitivity (relative value) | Maximum Density (D max) | Minimum Density (D min) |
|----------------|-------------------------------------|-------------------------|-------------------------|
| 30             | 100                                 | 3.3                     | 0.21                    |
|                | 380                                 | 3.3                     | 0.05                    |
|                | 390                                 | 3.3                     | 0.05                    |
|                | 100                                 | 3.2                     | 0.28                    |
| 35             | 345                                 | 3.1                     | 0.08                    |
|                | 340                                 | 3.0                     | 0.08                    |
|                | 100                                 | 3.3                     | 0.17                    |
|                | 240                                 | 3.3                     | 0.05                    |
|                | 245                                 | 3.2                     | 0.05                    |
|                | 100                                 | 3.3                     | 0.31                    |
| 40             | 535                                 | 3.2                     | 0.05                    |
|                | 590                                 | 3.2                     | 0.05                    |
|                | 100                                 | 3.2                     | 0.18                    |
|                | 205                                 | 3.2                     | 0.06                    |
|                | 205                                 | 3.2                     | 0.06                    |
|                | 100                                 | 3.2                     | 0.62                    |
|                | 445                                 | 3.2                     | 0.06                    |
| 45             | 455                                 | 3.1                     | 0.06                    |
|                | 100                                 | 3.2                     | 0.30                    |
|                | 280                                 | 3.1                     | 0.08                    |
|                | 270                                 | 3.1                     | 0.08                    |
|                | 100                                 | 3.3                     | 0.12                    |

| Experiment No. | Compound Having Formula (I) | Compound Having Formula (II) |
|----------------|-----------------------------|------------------------------|
|                | Amount (mg/kg emulsion)     | Amount (mg/kg emulsion)      |
| 51             | I - 10                      | (18.3)                       |
| 52             | I - 10                      | (18.3)                       |
| 53             | I - 12                      | (20.4)                       |
| 54             | I - 13                      | (20.4)                       |
| 55             | I - 13                      | (20.4)                       |
| 56             | I - 13                      | (25.0)                       |
| 57             | I - 13                      | (25.0)                       |
| 58             | I - 13                      | (25.0)                       |
| 59             | I - 14                      | (21.0)                       |
| 60             | I - 14                      | (21.0)                       |
| 61             | I - 14                      | (21.0)                       |
| 62             | I - 15                      | (28.8)                       |
| 63             | I - 15                      | (28.8)                       |
| 64             | I - 15                      | (28.8)                       |
| 65             | I - 16                      | (33.5)                       |
| 66             | I - 16                      | (33.5)                       |
| 67             | I - 16                      | (33.5)                       |
| 68             | I - 17                      | (32.2)                       |
| 69             | I - 17                      | (32.2)                       |
| 70             | I - 17                      | (32.2)                       |
| 71             | I - 18                      | (19.0)                       |
| 72             | I - 18                      | (19.0)                       |
| 73             | I - 18                      | (19.0)                       |

| Yellow Sensitivity<br>(relative value) | Maximum Density<br>(D max) | Minimum Density<br>(D min) |
|----------------------------------------|----------------------------|----------------------------|
| 410                                    | 3.3                        | 0.05                       |
| 405                                    | 3.3                        | 0.05                       |
| 100                                    | 3.2                        | 0.20                       |
| 2050                                   | 3.2                        | 0.07                       |
| 2100                                   | 3.2                        | 0.07                       |
| 100                                    | 2.9                        | 0.36                       |
| 205                                    | 2.9                        | 0.10                       |
| 200                                    | 2.9                        | 0.10                       |
| 100                                    | 3.0                        | 0.32                       |
| 520                                    | 3.0                        | 0.08                       |
| 510                                    | 2.9                        | 0.08                       |
| 100                                    | 3.2                        | 0.16                       |
| 190                                    | 3.2                        | 0.07                       |
| 175                                    | 3.1                        | 0.07                       |
| 100                                    | 3.2                        | 0.15                       |
| 170                                    | 3.2                        | 0.07                       |
| 175                                    | 3.2                        | 0.07                       |
| 100                                    | 3.1                        | 0.50                       |
| 2700                                   | 3.1                        | 0.07                       |
| 2600                                   | 3.0                        | 0.07                       |
| 100                                    | 3.2                        | 0.62                       |
| 500                                    | 3.2                        | 0.05                       |
| 515                                    | 3.2                        | 0.05                       |

| Yellow Sensitivity<br>(relative value) | Maximum Density<br>(D max) | Minimum Density<br>(D min) |
|----------------------------------------|----------------------------|----------------------------|
| 670                                    | 3.2                        | 0.09                       |
| 100                                    | 3.2                        | 0.18                       |
| 510                                    | 3.2                        | 0.07                       |
| 550                                    | 3.2                        | 0.07                       |

FIG. 2 shows characteristic curves wherein curves 2 and 3 correspond to Experiment No. 32 and 33 in Table 2.

### EXAMPLE 3

A silver chloride iodide bromide emulsion (iodine: 1.3 mol % and bromine 21.3 mol %) was fogged by formalin and the pH and pAg were adjusted to 5.6 and 6.7, respectively. This emulsion contained a rhodium salt which was added at formation thereof.

To the above mentioned emulsion, compounds represented by the formula (II) shown in the following

| Experiment No. | Compound Having Formula (I) | Compound Having Formula (II) |
|----------------|-----------------------------|------------------------------|
|                | Amount (mg/kg emulsion)     | Amount (mg/kg emulsion)      |
| 74             | I - 19                      | (18.4)                       |
| 75             | I - 19                      | (18.4)                       |
| 76             | I - 19                      | (18.4)                       |
| 77             | I - 20                      | (22.9)                       |
| 78             | I - 20                      | (22.9)                       |
| 79             | I - 20                      | (22.9)                       |
| 80             | I - 21                      | (25.9)                       |
| 81             | I - 21                      | (25.9)                       |
| 82             | I - 21                      | (25.9)                       |
| 83             | I - 22                      | (28.0)                       |
| 84             | I - 22                      | (28.0)                       |
| 85             | I - 22                      | (28.0)                       |
| 86             | I - 23                      | (30.7)                       |
| 87             | I - 23                      | (30.7)                       |
| 88             | I - 23                      | (30.7)                       |
| 89             | I - 24                      | (24.0)                       |
| 90             | I - 24                      | (24.0)                       |
| 91             | I - 24                      | (24.0)                       |
| 92             | I - 25                      | (22.0)                       |
| 93             | I - 25                      | (22.0)                       |
| 94             | I - 25                      | (22.0)                       |
| 95             | I - 26                      | (15.8)                       |
| 96             | I - 26                      | (15.8)                       |
| 97             | I - 26                      | (15.8)                       |

| Yellow Sensitivity<br>(relative value) | Maximum Density<br>(D max) | Minimum Density<br>(D min) |
|----------------------------------------|----------------------------|----------------------------|
| 100                                    | 3.2                        | 0.16                       |
| 420                                    | 3.2                        | 0.05                       |
| 420                                    | 3.2                        | 0.05                       |
| 100                                    | 3.0                        | 0.26                       |
| 320                                    | 2.9                        | 0.08                       |
| 315                                    | 2.9                        | 0.08                       |
| 100                                    | 3.0                        | 0.25                       |
| 760                                    | 3.0                        | 0.07                       |
| 740                                    | 3.0                        | 0.07                       |
| 100                                    | 3.1                        | 0.21                       |
| 290                                    | 3.1                        | 0.05                       |
| 280                                    | 3.1                        | 0.05                       |
| 100                                    | 3.0                        | 0.23                       |
| 195                                    | 3.0                        | 0.07                       |
| 180                                    | 2.9                        | 0.07                       |
| 100                                    | 3.0                        | 0.26                       |
| 950                                    | 3.0                        | 0.07                       |
| 810                                    | 3.0                        | 0.07                       |
| 100                                    | 3.3                        | 0.21                       |
| 670                                    | 3.2                        | 0.09                       |

Table 3 were added. Then, dyes represented by the formula (I), dispersions of couplers having the following formula (III) and a hardener were added in turn thereto. The products were applied to a triacetyl cellulose base. In order to compare, dyes represented by the formula (II), a dispersion of a coupler having the above mentioned formula (12) and a hardener were added in 45 turn to the above mentioned emulsion. The product was applied to a base. After drying these films were exposed to light through step-wedges under a yellow filter (Fuji Filter No. 12 ("Fuji" is registered trade mark)).

After exposing, the samples were developed with 55 using a color developing solution. The films were then treated by fixing, rinsing, bleaching, rinsing, hardening, rinsing and stabilizing in turn.

The results are shown in Table 3.

Table 3

| Experiment No. | Compound Having Formula (I) | Compound Having Formula (II) |
|----------------|-----------------------------|------------------------------|
|                | Amount (mg/kg emulsion)     | Amount (mg/kg emulsion)      |
| 98             | I - 3                       | (20.7)                       |
| 99             | I - 3                       | (20.7)                       |
| 100            | I - 24                      | (24.0)                       |
| 101            | I - 24                      | (24.0)                       |
| 102            | I - 25                      | (22.0)                       |
| 103            | I - 25                      | (22.0)                       |
|                |                             | II - 8 (400)                 |
|                |                             | —                            |
|                |                             | II - 8 (400)                 |
|                |                             | —                            |
|                |                             | II - 4 (400)                 |

| Yellow Sensitivity<br>(relative value) | Maximum Density<br>(D max) | Minimum Density<br>(D min) |
|----------------------------------------|----------------------------|----------------------------|
| 100                                    | 2.5                        | 0.30                       |
| 380                                    | 2.5                        | 0.10                       |
| 100                                    | 2.6                        | 0.25                       |
| 1200                                   | 2.6                        | 0.10                       |
| 100                                    | 2.6                        | 0.25                       |
| 1050                                   | 2.6                        | 0.11                       |

As is clear from the data contained in the above-mentioned Table 1-3, if the halogen accepting sensitizing cyanine dyes represented by the formula (I) are added together with the compounds represented by the formula (II) to the emulsion, direct positive silver halide emulsions (sensitive material) having a remarkably high yellow sensitivity and a comparatively low maximum density are obtained as compared with emulsions containing only the cyanine dyes.

What is claimed is:

What is claimed is:

1. A direct positive silver halide photographic emulsion comprising fogged silver halide and a combination of at least a sensitizing halogen accepting cyanine dye represented by the formula (I)



wherein Z and Z<sub>1</sub> each represents non-metal atoms necessary to complete a thiazole nucleus, an oxazole nucleus, a selenazole nucleus, a thiazoline nucleus, an oxazoline nucleus, a quinoline nucleus, an isoquinoline nucleus, a benzimidazole nucleus, or a 3,3'-dialkylindolenine nucleus, R and R<sub>1</sub> each represents an alkyl group or an aryl group, L<sub>1</sub>, L<sub>2</sub> and L<sub>3</sub> each represents a methine group, p and q each represents 1 or 2, n represents 1, 2 or 3, m represents 1 or 2, and X represents an anion, together with at least a compound represented by the following formula (II)



wherein Y represents  $=\text{CH}-$  or  $=\text{N}-$ ;  $\text{R}_2$ ,  $\text{R}_3$ ,  $\text{R}_4$  and  $\text{R}_5$  each represents a hydrogen atom, a hydroxy group, an alkoxy group, an aryloxy group, a halogen atom, a heterocyclic nucleus, an alkylthio group, heteracycliclothia group an arylthio group, an amino group, an alkylamino group, arylamins group a heterocycloamino group, an aryl group or a mercapto group; and  $-\text{A}-$  represents  $-\text{A}_1-$  or  $-\text{A}_2-$ , wherein  $-\text{A}_1-$  is



or 



with the proviso that when  $-A-$  represents  $-A_2-$ , at least one of  $R_2$ ,  $R_3$ ,  $R_4$  and  $R_5$  is a substituent containing a  $-SO_3M$  group, in which  $M$  is as described above.

**2. A direct-positive silver halide photographic emulsion according to claim 1, wherein the amount of the cyanine dye is within the range of 1-200 mg per 1 kg of the emulsion.**

3. A direct-positive silver halide photographic emulsion according to claim 1, wherein the amount of the compound represented by the formula (II) is within the range of 5-2000 mg per 1 kg of the emulsion.

4. A direct-positive silver halide photographic emulsion according to claim 1, wherein the ratio by weight of the cyanine dye to the compound (II) is 1:5-1:50.

5. A direct-positive silver halide photographic emulsion according to claim 1, wherein said heterocyclic nucleus formed by Z and Z<sub>1</sub> is a thiazole nucleus, an oxazole nucleus, a selenazole nucleus, a thiazoline nucleus, an oxazoline nucleus, a quinoline nucleus, an isoquinoline nucleus, a benzimidazole nucleus, or a 3,3'-dialkylindolenine nucleus.

6. A direct positive silver halide photographic emulsion according to claim 5, wherein the heterocyclic nucleus formed by Z and Z<sub>1</sub> is thiazole, 4-methylthiazole, 4-phenylthiazole, 5-methylthiazole, 5-phenylthiazole, 4,5-dimethylthiazole, 4,5-diphenylthiazole, 4-(2-thienyl)-thiazole, benzothiazole, 4-chlorobenzothiazole, 5-chlorobenzothiazole, 6-chlorobenzothiazole, 7-chlorobenzothiazole, 5-methylbenzothiazole, 6-methylbenzothiazole, 5-bromobenzothiazole, 5-phenylbenzothiazole, 5-methoxybenzothiazole, 6-methoxybenzothiazole, 5-ethoxybenzothiazole, 5,6-dimethoxybenzothiazole, 5-hydroxybenzothiazole, 6-hydroxybenzothiazole, naphtho(1,2)-thiazole, naphtho(2,3)-thiazole, naphtho(2,1)-thiazole, 4-methyloxazole, 5-methyloxazole, 4-phenyloxazole, 4,5-diphenyloxazole, 4-ethyloxazole, 4,5-dimethyloxazole, 5-phenyloxazole, benzoxazole, 5-chlorobenzoxazole, 5-methylbenzoxazole, 5-phenylbenzoxazole, 6-methylbenzoxazole, 5,6-dimethylbenzoxazole, 5-methoxybenzoxazole, 5-ethoxybenzoxazole, 5-hydroxybenzoxazole, 6-hydroxybenzoxazole, naphtho(1,2)-oxazole, naphtho(2,3)-oxazole, 4-methylselenazole, 4-phenylselenazole, benzoselenazole, 5-chlorobenzoselenazole, 5-methoxybenzoselenazole, naphtho(1,2)-selenazole, naphtho(2,1)-selenazole, thiazoline, 4-methylthiazoline, oxazoline, 2-quinoline nuclei selected from the group consisting of quinoline, 3-methylquinoline, 5-methylquinoline, 6-chloroquinoline, 6-chloroquinoline, 6-methoxyquinoline, 6-ethoxyquinoline, 6-hydroxyquinoline, and 8-hydroxyquinoline, 4-quinoline nuclei selected from the group consisting of quinoline, 6-methoxyquinoline, 6-methylquinoline, 6-chloroquinoline, 6-chloroquinoline, 6-fluoroquinoline, 8-fluoroquinoline, 6-hydroxyquinoline, 8-hydroxyquinoline, and 6-methylquinoline, 1-isoquinoline nuclei selected from the group consisting of isoquinoline, and 3,4-dihydroquinoline, 3-isoquinoline, 1,3-diethylbenzimidazole, 1,3-diethyl-5-chlorobenzimidazole, 1,3-diethyl-5,6-dichlorobenzimidazole, 1-ethyl-3-phenylbenzimidazole, 3,3'-dimethylindolenine, 3,3'-5-trimethylindolenine, or 3,3'-7-trimethylindolenine.

7. A direct-positive silver halide photographic emulsion according to claim 1, wherein said alkyl group for R and R<sub>1</sub> is a methyl group, an ethyl group, a propyl group, an isopropyl group, a butyl group, a hexyl group, a cyclohexyl group, a decyl group, or a dodecyl group.

8. A direct-positive silver halide photographic emulsion according to claim 1, wherein said alkyl group for R and R<sub>1</sub> is a substituted alkyl group selected from the group consisting of a hydroxyalkyl group, an alkoxyalkyl group, an acetoxyalkyl group, a carboxy radical-containing alkyl group, a sulfo radical containing alkyl group, an aralkyl group, and an allyl group.

9. A direct-positive silver halide photographic emulsion according to claim 8, wherein said hydroxyalkyl group is a 2-hydroxyethyl group or a 3-hydroxypropyl group, wherein said alkoxyalkyl group is a 2-methoxyethyl group, wherein said acetoxyalkyl group is a  $\beta$ -acetoxyethyl group or a  $\gamma$ -acetoxypropyl group, wherein said carboxy radical-containing alkyl group is a carboxy methyl group, a 2-carboxyethyl group, a

3-carboxypropyl group, a 2-(2-carboxyethoxy)-ethyl group, or a p-carboxybenzyl group, wherein said sulforadical-containing alkyl group is a 2-sulfoethyl group, a 3-sulfopropyl group, a 4-sulfobutyl group, a 2-hydroxy-1-sulfopropyl group, a 2-(3-sulfopropoxy)ethyl group, a 2-acetoxy-1-sulfopropyl group, a 3-methoxy-2-(3-sulfopropoxy)propyl group, a 2-(2-(3-sulfopropoxy)ethoxy)ethyl group, a 2-hydroxy-3-(3'-sulfopropoxy)-propyl group, a p-sulfobenzyl group, or a p-sulfophenethyl group, and wherein said aralkyl group is a benzyl group or a phenethyl group.

10. A direct positive silver halide photographic emulsion of claim 1, wherein said aryl group for R and R<sub>1</sub> is a phenyl group, a tolyl group, a naphthyl group, a methoxyphenyl group, or a chlorophenyl group.

11. A direct positive silver halide photographic emulsion of claim 1, wherein said X is a chlorine ion, a bromine ion, an iodine ion, a thiocyanic ion, a sulfonic ion, a perchloric ion, a p-toluenesulfonic ion, a methylsulfuric ion, or an ethylsulfuric ion.

12. A direct positive silver halide photographic emulsion according to claim 1, wherein said methine group for L<sub>1</sub>, L<sub>2</sub>, and L<sub>3</sub> is =C(-CH<sub>3</sub>)-, =C(-C<sub>2</sub>H<sub>5</sub>)-, =C(-C<sub>3</sub>H<sub>7</sub>)-, =C(-CH<sub>2</sub>C<sub>6</sub>H<sub>5</sub>)-, =C(-C<sub>6</sub>H<sub>5</sub>)-, =C(-alkoxy)-, =C(aryloxy)-, =C(-S-alkyl)-, =C(-O-acyl)-, =C(-amido)-, =C(-Cl)- and =C(-Br)-, and wherein the substituents of two methine groups of L<sub>1</sub>, L<sub>2</sub> and L<sub>3</sub> may bond together to form a ring represented by the following formula



wherein R<sub>6</sub> is a hydrogen atom or methyl group, and R<sub>7</sub> is a hydrogen atom, an alkyl group, an aryl group, a phenyl group or a furyl group.

13. A direct-positive silver halide photographic emulsion according to claim 1, wherein the cyanine dyes are selected from the group consisting of









and



14. A direct-positive silver halide photographic emulsion according to claim 1, wherein the compound (II) is selected from the group consisting of 55









and



15. A direct-positive silver halide photographic emulsion according to claim 1, wherein when  $R_2$ ,  $R_3$ ,  $R_4$  and  $R_5$  represent a heterocyclic nucleus it is selected from the group consisting of a morpholinyl nucleus and a pyperidyl nucleus, and wherein  $R_2$ ,  $R_3$ ,  $R_4$  and  $R_5$  repre-

sent a heterocyclic amino group it is selected from the group consisting of a 2-benzothiazoleamino group and a 2-pyridylamino group.

\* \* \* \*

35

40

45

50

55

60

65